

## UNITED STATES PATENT OFFICE

1,958,311

## LITHOGRAPHIC INK COMPOSITION

John V. Mehl, Union City, N. J.

No Drawing. Application August 16, 1932,  
Serial No. 629,082

1 Claim. (Cl. 134—35)

This invention relates to improvements in lithographic ink compositions and has for an object the provision of an improved lithographic ink which eliminates the necessity for wetting the lithographic plate between each printing operation.

A further object of this invention is the provision of an improved lithographic ink which may easily be applied to the prepared plate and which 10 will only adhere to the desired portions of the plate so that a sharply defined print may be made by the plate.

In the lithographing art the plate, consisting of a flat stone, or a zinc or aluminum sheet, has the 15 design formed thereon by coating or impregnating the surface of the plate with a greasy or waxy material, by which such portion of the plate is made repellent to water but with an affinity for greasy or waxy ink, while the remaining portions 20 of the surface of the plate will take on a thin layer of water which will then repel greasy or waxy ink.

Various methods are used in applying the design to the surface of a plate, such as by drawing 25 in reverse directly on the surface of the plate by hand with a greasy or waxy crayon, or by pen or brush, with liquid greasy ink, or by transferring the same from paper or from engraved plates or woodcuts, or from photographic plates upon 30 which the design has been formed by a coating of greasy or waxy material. Whichever method is used to form the subject matter upon the plate, the principle of the art of printing from lithographic plates is the same, which is the chemical 35 affinity of the greasy or waxy material coated or impregnated in the plate, for substances of the same nature in the ink, and the repugnance of such substances for water, by which the design on the plate will repel a coating of water but will take 40 a coating of the ink, and the uncoated portions of the plate will take a coating of water, which will prevent the ink from adhering to such water-coated portions.

The method now in use for printing from lithograph-plates requires the prepared plate to be 45 first coated with a film of water, which adheres to the portions of the plate free from the greasy material forming the designs thereon, and secondly, applying a coating of greasy ink to the plate, 50 which will adhere to and cover the design on the plate but will be repelled by the water coating. A sheet of paper or other flexible material then being placed upon the plate will take up the greasy ink from the design thereon, thus producing a 55 print of the design upon the paper. Such method

requires the repetition of a water coating and an ink coating successively applied to the plate for each printing.

Still another object of the invention is the provision of a lithographic ink consisting of a material having an affinity for greasy substances, and other material repellent to greasy substances. These objects are accomplished by incorporating in the usual greasy lithographic ink a grease-repellent liquid consisting of a solution of sodium 60 hyposulfite, glycerine, rubber cement, and nicotine, and forming an emulsion of the said liquid with the ink. The most important of these ingredients is the sodium hyposulfite, which holds the liquid on the surface of the ink, and the nicotine which is a repellent to the greasy substance 65 in the ink will be deposited upon the portions of the plate not covered by the coating forming the design. The glycerine prevents drying of the solution in the ink, and the rubber cement renders 70 the solution tacky and prevents piling of the ink 75 upon the plate.

While the proportions of these substances may be varied, the most satisfactory results are accomplished by the following proportions by 80 weight: With one pound of the usual greasy lithographic ink is mixed one-half ounce of a saturated solution of sodium hyposulfite, one-half ounce of glycerine, one-half ounce of rubber cement, and one-half ounce of nicotine in solution 85 with one-quarter ounce of benzol as a vehicle to produce an emulsion with the ink. The aforesaid substances are thoroughly mixed, forming a jelly-like solution which is then worked in with the ink to form minute globules of the ink interspersed 90 with minute globules of the solution. While the solution is difficult to combine with the ink, the addition of a small quantity of benzol readily permits an emulsion being formed with the ink; the benzol being volatile, evaporates from the solution 95 as the same is worked in with the ink.

The ink thus prepared may be applied to the lithographic plate in the usual manner by means of a roller, which, passing over the plate, will deposit a thin film of the greasy ink upon the 100 design formed on the plate, and on the remaining portions of the plate the solution separating from the ink will be deposited, thus producing in one operation what has heretofore been accomplished in two operations, namely, the wetting 105 of the plate, followed by the inking of the plate. After the plate has been inked with the improved material the paper, leather or other flexible material may be applied to the surface of the plate and the inked coating on the plate in the form 110

of the design, will be transferred to the paper, leather or other material.

In the printing of the multi-copies in accordance with the present invention, the portions of the plate not covered by the greasy design are first wetted with water or with a thin solution of nicotine, after which the improved ink is applied thereto as hereinbefore described. The first print is then made from the plate. For each subsequent printing it is unnecessary to again wet the plate, as the improved ink has incorpo-

rated therein the substance having an affinity for the uncoated portions of the plate.

What is claimed is:

A lithographic ink consisting of an emulsion of a greasy ink, a saturated solution of sodium hyposulfite, glycerine, rubber cement, and nicotine in the proportion of substantially one pound of the greasy ink to one-half ounce of each of the other substances. 80

JOHN V. MEHL. 85

15

90

20

95

25

100

30

105

35

110

40

115

45

120

50

125

55

130

60

135

65

140

70

145

75

150